

July 26, 1927.

J. R. LONG

1,636,748

PAPER INSULATED ELECTRIC CONDUCTOR

Filed Jan. 12, 1926

Fig. 1



Fig. 2



INVENTOR.  
John R. Long.  
BY Edward A. Lawrence  
his ATTORNEY.

## UNITED STATES PATENT OFFICE.

JOHN R. LONG, OF TARENTUM, PENNSYLVANIA.

PAPER-INSULATED ELECTRIC CONDUCTOR.

Application filed January 12, 1926. Serial No. 80,814.

The object which I have in view is the provision of a paper insulated electric conductor which will be able to carry higher voltage and at reduced loss of current, and which will be more flexible for bending and free from injury therefrom.

In the present practice the electric conductors, such as cables and wires are tautly wound with a plurality of plies of strips of paper, paper made from old rope fibres being preferably employed to obtain the desirable tensile strength and exterior smoothness necessary to pass through the former or die of the winding machine. Paper made from old rope fibres is used owing to the high cost of new manila fibre. Old rope fibre is usually contaminated with foreign matter, such as grease, oils, metals, sand, salt, &c., that have accumulated in its previous service, and the presence of such foreign matters impairs the dielectric properties of the insulation and increases the current loss.

Under the present practice it is impossible to remove these impurities from old rope stock, and the supply obtainable is not only becoming scarcer but is growing more contaminated; and the rope stock is often adulterated in manufacture, frequently carrying a large percentage of sisal, or other inferior fibres.

In addition to the current loss due to impurities in the old rope paper, a conductor wrapped with the same shows a certain loss in flexibility owing to the friction between the surfaces of tightly wrapped layers of the same material.

As a substitute for old rope paper, I have employed paper made from spruce pulp cellulose, so treated as to become mechanically pure, thereby obtaining a higher degree of insulation; but the frictional means employed for winding and tauting the paper about the conductor tends to accumulate a certain amount of fuzz, or lint, resulting in a roughness of surface which interferes with the passage of the cable through the former or die employed to insure a smooth, uniform external surface to the cable.

Again, the wood pulp paper presents like surfaces in contact which cause internal friction in the insulating envelope, causing the conductor unduly to resist bending and resulting in injury to the insulation from bending.

Attempts have been made to employ paper

composed of a mechanical mixture of cellulose, such as wood pulp or jute fibres and old rope fibres, but the impurities in the old fibres impair the insulating properties, and the fault of excess friction between surfaces of like material evinces itself.

In my present invention I provide an electric conductor having an insulating envelope formed of one or more layers of spirally wound strips of paper whose opposite surfaces are formed of different materials, thus minimizing the friction.

For instance the paper covering may be formed of spirally wound strips of paper whose body is composed of wood cellulose, and one of whose surfaces, preferably the outer surface is formed by a layer of vegetable fibre with the majority of the fibres laid in the general direction of the length of the paper strip to increase its tensile strength. Such vegetable fibres as those of cotton, rice, hemp, ramie, jute and the like may be used.

Thus also I may form the one layer or the body of the paper of jute fibre and the other layer of old rope or other vegetable fibres.

I prefer to use a mechanically pure Swedish spruce cellulose as the stock for the body of the paper.

For the surface layer of vegetable fibre I may use such fibres as those of cotton, rice, hemp, ramie, jute and the like, but I prefer to employ old rope fibre.

In the accompanying drawings, Fig. 1 is a broken perspective showing a composite wire cable wrapped with three layers of insulating paper in accordance with my present invention, and Fig. 2 is a view in perspective of a short strip of said paper, the two exterior surfaces being shown separated in an arbitrary manner for the sake of illustration.

In the drawing 1 represents the wires which form the electric conductor or cable and 2 represents the insulating covering comprising three spirally wound layers 2<sup>a</sup>, 2<sup>b</sup>, 2<sup>c</sup>.

The cable or wire is wound with this composite paper, preferably having a body of mechanically pure wood or jute cellulose and one surface of rope fibre with the rope fibre surface on the outside, and in the finished conductor the frictional contact is not between surfaces of like material, but between a surface of cellulose material and a

surface of rope or other vegetable fibre, and thus the friction is reduced to a minimum, resulting in a conductor of greatly increased flexibility and one whose insulating covering will not wear out or be functionally impaired from bending.

The wound cable will also present a smooth, uniform surface which will pass easily through the former or die without abrasion.

My improved paper is also cheaper than paper made wholly of new manila hemp or old rope fibres.

What I desire to claim is:—

- 15 1. An electric conductor having a paper insulating envelope formed of one or more spirally wound layers of paper of composite character having opposite surfaces formed of different materials.
- 20 2. An electric conductor having a paper insulating envelope formed of a plurality of layers of spirally wound paper of composite character having its opposite surfaces

of different material to minimize friction between the layers.

25 3. An electric conductor having a paper insulating envelope formed of spirally wound layers of paper of composite character having one surface of cellulose material and the other surface of vegetable fibres 30 to reduce the friction between the layers.

4. An electric conductor having a paper insulating envelope formed of spirally wound layers of paper of composite character having one surface of cellulose material and the other surface of manila fibre.

5. An electric conductor having a paper insulating envelope formed of a plurality of spirally wound layers of paper of composite character having one surface of cellulose material and the other surface of old rope fibre to reduce the friction between the layers.

Signed at Pittsburgh, Pa., this 31st day of December, 1925.

JOHN R. LONG.